

## UNITED STATES PATENT OFFICE.

GEORGE L. NORRIS, OF SUMMIT, NEW JERSEY, ASSIGNOR TO VANADIUM CORPORATION OF AMERICA, A CORPORATION OF DELAWARE.

## STEEL ALLOY.

No Drawing.

Application filed January 19, 1927. Serial No. 162,208.

This invention relates to alloy steels and particularly to steels containing silicon in somewhat greater proportion than the ordinary steels of commerce.

5 The addition of silicon to steel is known to have a beneficial effect. Steels containing relatively high proportions of silicon have, however, the disadvantage of being very sensitive to heat treatment, that is to say, 10 the temperature range within which certain desirable physical properties can be obtained by quenching and drawing is relatively limited. Moreover, the silicon steels heretofore known lack the high tensile 15 strength, toughness and resistance to alternating stresses and shocks which are essential to meet the conditions in certain uses of such steels.

It is the object of the present invention to 20 provide an improved silicon steel which is adapted especially for use in various structural parts of boilers, pressure tanks, stills and hulls, engine and machinery parts, springs, bolts and tools, and is designed particularly to meet the peculiar stresses to 25 which such parts are subjected.

Other objects and advantages of the invention will be apparent as it is better understood by reference to the following specification.

30 in which the preferred compositions are described.

I have discovered that the addition of vanadium to silicon steels, and particularly to steels of the composition hereinafter described, results in a very material improvement in the quality and characteristics of the product. The vanadium increases the ratio of elastic limit to tensile strength, the ductility and shock resistance of the steel, 40 thus making it suitable for various uses to which such steel has not been well adapted heretofore. The vanadium also overcomes the well known tendency of silicon to cause separation of carbon in the steel in the form of graphite and consequent injury to the physical properties of the steel. As the result of the improvement it is possible to construct parts of lighter weight with the same or greater physical strength than parts made 45 of steel as heretofore known. The addition of vanadium results, therefore, in the production of steels which afford considerable

commercial advantage with the additional factor of safety provided by the greater strength of the steels.

55 In carrying out the invention, I prefer to employ silicon in the proportions of 0.40% to 2.00% and manganese from 0.20% to 0.60%, together with vanadium in the proportions of 0.05% to 0.50%. The amount of carbon in the steel can be varied within a relatively wide range. A low carbon steel may include from 0.10% to 0.30% of carbon which may, however, range as high as 1.0% providing a steel having the characteristic qualities of steels with relatively high carbon content. The proportions of silicon, manganese and vanadium may likewise vary within the comparatively wide ranges indicated 65 to produce steels having the desired qualities 70 and characteristics to adapt them for the special uses for which they are intended.

I have discovered also that the steels as described may be further improved by the addition of nickel preferably in amount not 75 exceeding 1.5% or copper not in excess of 0.5%. These elements are especially beneficial in increasing the corrosion resistance of the steel without adversely affecting the physical properties which result from the 80 presence of silicon and vanadium.

The improved steels can be produced by any of the well known steel-making processes. The silicon and vanadium can be added in the form of ferro-alloys in the 85 usual manner to the ladle during the tapping of the steel from the furnace, or in the case of electric furnace and acid open hearth furnace steel, the ferrosilicon and ferrovanadium may be added to the molten bath of 90 steel in the furnace with a short interval, sufficient to allow them to melt, before tapping. It is desirable to reladle the steel, that is, pour from one ladle into another before casting the steel into molds. This is particularly desirable when the ferrosilicon and ferrovanadium are added to the ladle in order to secure greater uniformity, lessen the possibility of segregation, and reduce the amount of piping in the ingot, all of which 100 are influenced by the large percentage of silicon added.

I have also discovered that steels containing silicon can be improved with respect to

physical properties and particularly as to the ratio of elastic limit to tensile strength, ductility and shock resistance by the addition of molybdenum in suitable proportions to a steel having the composition, for example, of silicon 0.40% to 1.25%, manganese 0.20% to 0.40%, and carbon 0.10% to 0.30%. To such a steel I find it advantageous to add from 0.10% to 1.00% of molybdenum to obtain the desired improvement in the characteristics mentioned.

It is to be understood that the steels as described may include the usual impurities such as sulphur and phosphorus in the proportions permitted by standard steel specifications or in amounts which are not detri-

mental to the qualities of the steel and that other elements may be present likewise either as inert elements or for the purpose of further improving the physical properties of the steel. Various changes may be made, therefore, in the composition as described without departing from the invention or sacrificing any of the advantages thereof.

I claim:—

A steel alloy consisting of silicon 0.40% to 2.00%, vanadium 0.05% to 0.50%, manganese 0.20% to 0.60% and carbon 0.10% to 1.00%, the balance being iron with the usual impurities of commercial steel.

In testimony whereof I affix my signature.

GEORGE L. NORRIS.

25

30